

## UNITED STATES PATENT OFFICE

2,163,583

## TREATMENT OF MAGNESIUM AND ITS ALLOYS

Robert W. Buzzard, Kensington, Md.

No Drawing. Application November 26, 1937,  
Serial No. 176,651

6 Claims. (Cl. 148—6)

(Granted under the act of March 3, 1883, as  
amended April 30, 1928; 370 O. G. 757)

This invention relates to the forming of protective coatings on magnesium or its alloys.

It is an object of this invention to regulate the pH of a bath so as to form on magnesium or its alloys a protective coating that has exceptionally good mechanical and corrosion-resisting characteristics.

It has been proposed in United States Patent 1,947,122 to treat magnesium or magnesium alloys with a solution of a dihydrogen phosphate and a salt of chromic acid in order to form an adherent coating on the surface of the metal to protect the same against corrosion. A solution prepared in accordance with this patent gives approximately a neutral bath slightly on the acid side, however the pH of this bath is not adjusted and regulated and is at all times higher than applicant's bath herein set forth. This bath produces a light gray coating on Dowmetal "H" alloy consisting of 6 percent aluminum, 2 percent zinc, and the remainder magnesium. I have found that a distinct improvement in and a superior corrosion resistant coating on magnesium and its alloys can be obtained by forming the coatings on the metal surfaces in a bath containing phosphoric acids and chromic acids or compounds thereof with the pH adjusted to and maintained within the range of pH 0.5 to pH 3.5. The resultant coating as produced by my process varies from a deep black to a greenish black on "H" alloy denoting a difference in physical properties from the specific coating referred to in the aforementioned patent. Further, a corrosion test of "H" alloy specimens disclosed that the specimens prepared in accordance with the patent failed 75 percent of the coating in 200 hours, whereas, the specimens treated in accordance with my method herein described failed 10 percent of the coating over the same period.

The bath of my improved process consists essentially of solutions of phosphoric acid and chromic acid adjusted to a pH within the range of pH 0.5 to pH 3.5 by a compound giving the basic reaction. To adjust the pH I add hydroxide, preferably ammonium hydroxide, however, either sodium or potassium hydroxide may be used, to the solution until the proper value is obtained.

Practically any concentration of chromic acid and phosphoric acid has been found satisfactory as long as the pH is adjusted, the useful concentration apparently being limited only by the solubility of the salts used, although some concentrations are preferable for particular alloys and for particular types of coatings.

The article to be coated is thoroughly cleaned, a clean surface being essential to the formation of

good coatings. Degreasing, electrolytic cleaning, acid cleaning, and acid pickling previous to coating all aid in the preparation of the surface of the metal for a good coating, although a number of known pretreatments may be used to clean the metal. After cleaning and washing, the article to be coated is immersed in the solution heated to approximately the boiling point of water or above. The time of treatment depends upon the strength of the solution and the quality of coating desired. Coatings have been produced by immersing the article for periods varying from 1 minute to 2 hours.

As an example, an article of magnesium alloy is first degreased, washed, electrolytically cleaned, washed, cleaned by acid dip, washed and then immersed for 30 minutes in a bath containing 90 grams/liter chromic acid and 80 grams/liter phosphoric acid adjusted to pH 1.5 with ammonium hydroxide, the bath being maintained during treatment at a temperature substantially equivalent to or above the boiling point of water. The bath, if and when necessary, is regulated and maintained at the proper pH by adding either phosphoric or chromic acid to the bath.

The invention herein described and claimed may be used and/or manufactured by or for the Government of the United States of America for governmental purposes without the payment of any royalties thereon or therefor.

I claim:

1. A method of forming a protective coating on magnesium and magnesium alloys, comprising immersing the metal to be coated in a bath containing chromic acid and phosphoric acid adjusted to a pH within the range of pH 0.5 to pH 3.5.

2. A method of forming a protective coating on magnesium and magnesium alloys, comprising immersing the metal to be coated in a bath containing substantially 90 grams per liter chromic acid, 80 grams per liter phosphoric acid and sufficient ammonium hydroxide to adjust the bath to a pH 1.5 and maintaining a constant pH of 1.5 by adding an acid selected from the group of phosphoric acid and chromic acid.

3. A method of forming a protective coating on magnesium and magnesium alloys, comprising immersing the metal to be coated in a bath containing chromic acid, phosphoric acid and hydroxide selected from the group ammonium hydroxide, sodium hydroxide and potassium hydroxide for adjusting the bath to a pH within the range pH 0.5 and pH 3.5, said bath being maintained during treatment at a temperature substantially equivalent to or above the boiling point

45

50

55

55

of water and being maintained at all times within the range pH 0.5 and pH 3.5 by adding an acid selected from the group of phosphoric acid and chromic acid.

5 4. A method of regulating a bath for treating magnesium and magnesium alloys comprising making a bath containing chromic acid and phosphoric acid, adjusting said bath within the range of pH 0.5 and pH 3.5 and maintaining at all times the bath within the range of pH 0.5 and pH 3.5.

10 5. A method of forming protective coatings on magnesium and magnesium alloys and for regulating a bath for treating the metal, comprising making an aqueous solution containing chromic acid and phosphoric acid, adjusting said solution within the range of pH 0.5 and pH 3.5 by adding a water soluble substance selected from the group of alkaline salt and hydroxide to the solution and

maintaining the resultant bath at all times within the range of pH 0.5 and pH 3.5 by adding an acid selected from the group of chromic acid and phosphoric acid.

6. A method of forming protective coatings on 5 magnesium and magnesium alloys and for regulating a bath for treating the metal, comprising making an aqueous solution containing chromic acid and phosphoric acid, adjusting said solution within the range of pH 0.5 and pH 3.5 by adding 10 hydroxide selected from the group of ammonium hydroxide, sodium hydroxide, and potassium hydroxide to the solution and maintaining the resultant bath at all times within the range of pH 0.5 and pH 3.5 by adding an acid selected from 15 the group of chromic acid and phosphoric acid.

ROBERT W. BUZZARD.